

G. BLENIO.

AEROPLANE ELEMENT AND PROCESS OF MAKING SAME AND PRODUCT OF SAID PROCESS.  
APPLICATION FILED JAN. 11, 1918.

1,427,941.

Patented Sept. 5, 1922.

Fig. 1.



Fig. 2.



Inventor

Guido Blenio.

Witness

John L. Cardeworth Dawson. By W. G. Elroy,  
his Attorney

## UNITED STATES PATENT OFFICE.

GUIDO BLENIO, OF NEW YORK, N. Y., ASSIGNOR, BY MESNE ASSIGNMENTS, TO BLENIO PAINT & PRODUCTS CORPORATION, OF NEW YORK, N. Y., A CORPORATION OF DELAWARE.

AEROPLANE ELEMENT AND PROCESS OF MAKING SAME AND PRODUCT OF SAID PROCESS.

Application filed January 11, 1918. Serial No. 211,419.

To all whom it may concern:

Be it known that I, GUIDO BLENIO, a subject of the King of Italy, residing at New York, in the county of New York and State 5 of New York, have invented certain new and useful Improvements in Aeroplane Elements and Processes of Making Same and Products of said Processes, of which the following is a specification.

- 10 This invention relates to aeroplane elements and processes of making same and products of said processes; and it comprises as a new article an airship plane of trussed cellular wooden construction enclosed in 15 fabric under tension, said fabric being impregnated with fireproofing salts and carrying a facing layer of relatively damp or hygroscopic flame-proof material shielded and sealed in against access of air by one 20 or more thin impermeable films of waterproofing material, said films being further protected by a varnish or paint coating; said cellular wooden construction being also advantageously protected in similar manner; 25 and it also comprises a method of making a protected fabric for aeroplanes and other purposes wherein a fabric is first impregnated with fireproofing salts somewhat dried, coated with a colloid hygroscopic material, 30 such as glue, sharply dried and coated with a thin waterproofing film, such as pyroxylin, the whole finally being painted or varnished; and it further comprises as a new article a layer of textile fabric impregnated with fire- 35 proofing salts and having one or both sides carrying a flame-proof colloid layer of more or less damp nature, such as glue containing hygroscopic materials, and faced with a thin layer of waterproofing material, such 40 as pyroxylin, this layer being in turn, if desired, mechanically protected by a coating of paint or varnish; all as more fully hereinafter set forth and as claimed.

Planes for aerial work are built of a 45 trussed cellular wooden framework with a sheet of fabric stretched over and covering both sides. Much is required, and more is desired, of this fabric. It must be strong, light and taut; and the tautness must not 50 vary according to the humidity. It should

be impermeable to air and water. And it is highly desirable that it be fireproof as well. Canvas (either linen or cotton) is the textile fabric ordinarily employed and to impart it the other qualities desired a wide 55 variety of "dopes" have been proposed. For the most part, these are ordinarily waterproofing compositions and materials, rubber, pyroxylin, varnishes, etc. Unfortunately, most of the materials used for waterproofing are quite as combustible as the canvas itself, and often more so. Pyroxylin, in its various commercial forms of celluloid, collodion cotton, gun cotton, etc., is one of the best of these waterproofing materials for aeroplane work, and is largely used, but of course it is highly combustible. In the effort to obviate its inflammability it is often used admixed with various hygroscopic salts (calcium chlorid, etc.) or mineral 60 matters; but in these admixtures the good qualities of the pyroxylin for the present purposes are largely forfeited. The same applies to most of the ordinary varnishes—the less inflammable they are, as a rule, the 65 less efficient they are for waterproofing.

One of the best materials, probably, is cellulose acetate which is not readily inflammable—no more so than canvas itself. In any event, and which when used on the 70 canvas fills up the pores, and by reducing the air content of the fabric reduces its inflammability. Any really efficient fireproofing composition must contain either moisture or ammonia salts; water vapors and ammonia gas being the only really efficient, protectively acting fire extinguishing means. Any insoluble solid mineral material, as such, does not detract from inflammability. Very many propositions have been made for 75 using moist materials in connection with waterproofing substances to produce compound dopes which were both waterproof and fireproof. For obvious reasons, however, these have not been satisfactory.

For fireproofing purposes, as stated, the material should contain either water or ammonia or both. There are very many salts which contain water of crystallization. Ordinary crystallized sodium sulfate or 80

Glauber's salt, for instance, contains more than half its weight of water of crystallization. Borax, alum, sulfate of alumina, sodium phosphate, etc., also contain much water of crystallization. Calcium chlorid, magnesium chlorid and many other salts are what are known as deliquescent. They tend to take up water from the air with formation of moist or liquid material. Many other salts contain ammonia in large amounts, as for instance ammonium sulfate, ammonium phosphate, etc., and some contain both water and ammonia, as for instance "microcosmic salt" (sodium ammonium phosphate), ammonia magnesium phosphate, etc. Any of these salts is an efficient fireproofing material when used to impregnate vegetable fabrics for the reason that when heat is applied flame stifling vapors are evolved. But they all have the objection that their relation to the humidity of the atmosphere is constantly varying; in dry weather they tend to lose moisture and in damp weather they tend to take it up. There are very many other materials of organic origin which are more or less fireproof in the sense that they are damp. Ordinary glue does not burn readily and when it is moist resists flame very well.

In the present invention I utilize the stated principles and materials to produce airship planes which have the desired combination of properties; being both weather or waterproof and flame-proof in the sense that they will not take fire from burning gasoline or incendiary projectiles, etc. To do this, in lieu of trying to make one single, "dope" which can be applied to the aeroplane surface and will at once produce all the desired results, I use the various materials in a methodical way so as to produce what may be termed a laminated or built up product in which the textile fabric itself is merely one layer or element. In so doing, I ordinarily apply the layer of textile fabric to the trussed wooden structure and make it as taut as may be. I then impregnate the fabric with a solution of fireproofing salts. While almost any hygroscopic salt, salt containing water of crystallization or ammonium salt may be used, in practice I find ammonium phosphate advantageous. In order to produce a more or less gelatinous character of the impregnant in the fabric and prevent any possible segregation in crystalline form I usually employ with the ammonium phosphate more or less aluminum sulfate. This gives me a mixture containing some sulfate of ammonia and some phosphate of alumina. This mixture I apply to the fabric with the aid of a brush or a spray, taking care that the fabric is wet completely through. The fabric is next dried but not absolutely so; I do not wish to produce a crystallization of dry material in the fabric or to drive off water of crystallization and ammonia. I merely wish it dry enough for the next coating. On the dried surface I next apply a layer of thick glue solution containing fireproofing salts, such as ammonium phosphate, in solution. It should also contain something hygroscopic, such as calcium chlorid, glycerin, sugar, etc. This layer I now dry in place, drying rather sharply so as to produce a dry surface while not expelling all the moisture from the interior. To this dried surface I next apply a thin or film coating of a good weather-proof material. A pyroxylin solution is advantageous for this purpose. The pyroxylin may be dissolved in amyl acetate, acetone or any other suitable quick drying solvent. On evaporation of the solvent the fabric and the glue layer, both of which are somewhat moist, though not very much so, are effectually sealed in by the pyroxylin while the pyroxylin layer itself is so thin as to be not readily inflammable. In order to avoid possibility of any bare spaces it is in general advisable to apply the desired amount of pyroxylin as a number of successive very thin films rather than as one coat, the coating being dried before each new application.

As so far stated, it will be observed that the cellular frame is completely enclosed in a layer of fabric which is somewhat moist and has been fireproofed by various salts. This fabric in turn is enclosed by a layer of an uninflammable glue also containing some moisture; and in turn this glue layer is enclosed by a continuous very thin film of waterproofing composition. This film seals in everything; there is no possibility of evaporation from the glue layer, the fabric or the enclosed space within the cellular framework. In order to perfect still further this sealing in effect I find it better to apply the successive coats of pyroxylin varnish with a thin spacing layer of glue between them. This obviates in large measure osmotic transference of moisture.

The application of moist materials to the canvas tautens it and since the amount of moisture must remain constant because of the sealing in, the tightness will not vary with weather or other conditions. I have therefore produced an article which is fire-proof, since no application of flame will produce any substantial results on the tenuous pyroxylin films or the underlying fire-proof materials. Glue, which is a very strong material, adds structural strength to that of the fabric. Completely dried glue is of course a strong but somewhat brittle material; but in my complete article there is enough softening water present for fire-proofing purposes to obviate this brittleness while there is not sufficient to detract from the mechanical strength. For mechanical protection of the thin waterproofing film I

ordinarily finally apply a thin coating of a good paint or varnish, such as a spar varnish. An ordinary limit for the weight of aeroplane facings is about 7 ounces per 5 yard, and I can produce all the required strength, with the other desirable results stated, within this limit by the use of a 4-ounce fabric carrying not to exceed 3 ounces of my various other materials.

10 In a specific embodiment of the present invention in fireproofing and protecting an aeroplane element, such as the wing surface, I may proceed as follows: Presuming the trussed wooden framework to be assembled 15 and ready for treatment I first brush it over thoroughly with a solution which I may here call No. 1. This solution I make by taking an ammonium phosphate solution neutral to litmus and of 15° Bé. and adding to it sufficient aluminum sulfate to bring the density to about 17° Bé. By reason of the interaction of the phosphate with the alumina there is produced a composition of a more or less thick character. This composition I dilute 20 with water to a density of around 7° Bé. With this diluted No. 1 I may impregnate the woodwork. The fabric is fixed to the woodwork in the usual way, being stretched as taut as possible. I next brush it thoroughly 25 with the diluted No. 1 composition, seeking to wet the fabric thoroughly therewith. This produces additional tensioning of the fabric and enhances the tautness. The plane is next dried to some extent. Since I desire to retain moisture, I do not dry 30 thoroughly. The next treatment is with a fireproofing mechanically strong gelatin or glue. This composition, which I may call No. 2, I usually make by taking good strong 35 glue or gelatin and swelling it in water for several hours, say over night. This swelled glue is next melted an a hygroscopic, softening material incorporated. Glycerin does very well. For each pound of swelled glue 40 I may use, say, two ounces of glycerin. It is desirable also to add an antiseptic since in use this composition will of course remain more or less damp. A good antiseptic for this purpose is salicylic acid. I may use 45 about one-fourth of an ounce for each pound of swelled glue. In swelling the amount of water which the glue will take up varies somewhat but ordinarily the glue takes up three times its weight of water. With this 50 glue solution I incorporate a certain amount of fireproofing salts. For example, I add to 3 parts of this glue solution 1 part of composition No. 1 of 17° Bé. The mixture will have a density of about 6° Bé. With this 55 No. 2 composition I next coat all the exposed surfaces, using one or more coats applied with a brush or spray as may be most convenient. The coated plane is next dried somewhat. It is advantageous now to apply 60 one or more thin coats of the glue solution with the addition of the No. 1 composition. The coated plane is now sharply dried; that is I dry at a rather high temperature but not for a long time, the effort being to make the outer surface absolutely dry in order to 65 receive the next coating, but not to drive out the moisture from the interior of the coating or from the fabric. The sharp dried surface now receives a thin coating of any 70 convenient waterproofing composition. Py- 75 roxylin, or collodion cotton dissolved in amyl acetate and thinned down with acetone is convenient. It is best to apply several very thin brush coats, drying between each coating in order to be able to attain an absolutely 75 impervious sealing film without using too much material. In the case of pyroxylin it is highly undesirable that the total thickness of this sealing film shall be very great. After this pyroxylin film is applied it is 80 advantageous to apply a thin coat of the glue solution, using for this purpose solution with the addition of the fireproofing salts or No. 1 composition. This layer of glue should be 85 very thin. After its application it is dried 90 sharply and another layer of pyroxylin applied; and so on, giving as many alternate thin coats of pyroxylin and glue as may be desired. Finally the whole assemblage is 95 best painted or varnished to give mechanical protection. A good spar varnish is suitable for this purpose.

It will be observed that in the article produced as just described fireproofing is attained by the use of fireproofing salts and 100 moisture in the glue. The glue has enough hygroscopic agent (glycerin in the example given) to keep it soft and pliable without forfeiting mechanical strength. The layer 105 of glue really forms a mechanical element in the assemblage. This glue is preserved from mildewing, molding, fermenting, etc. by the antiseptic, the salicylic acid. And the whole assemblage is shielded from the action 110 of air by the waterproofing composition. The principal element in the fireproofing of the assemblage is really the glue layer; the fireproofing of the fabric while useful not being so important. For the glue layer 115 protects the fabric against access of flame. In one embodiment of my invention I may omit fireproofing the fabric altogether. As however the fabric in this situation would become moist and would be exposed to decay I advantageously impregnate it thoroughly 120 with beeswax, paraffin, pitch, asphalt, etc. Or it may be impregnated with rubber and cured. I find it best in this modification of my invention to use a good grade of beeswax or ceresin. This adds considerably 125 to the mechanical strength of the cloth treated and permits the use of a lighter fabric for the same strength. Of course the fabric may be impregnated with fireproofing salts prior to impregnation with beeswax or 130

ceresin; but it is more convenient ordinarily to omit this fireproofing. Presuming the fabric has been impregnated with beeswax, either in a molten state or dissolved in a solvent, the No. 2 composition is applied as before and the various other coatings applied in the order stated.

In the accompanying drawings I have shown, more or less diagrammatically, an airship plane and a section of the covering illustrating my invention. It this showing

Figure 1 is a longitudinal section through an aeroplane wing; and

Figure 2 is a vertical section through one sheet of fabric etc. on a greatly enlarged scale.

In Figure 1, element 1 is the usual trussed wooden framework carrying a canvas, linen, etc. textile fabric 2 which has been treated in accordance with the described invention. It is stretched tautly over the frame in the usual way with its ends abutting as at 3, and is provided with the overlapping section of fabric 4 which is also treated in accordance with the present invention. The fabric is stitched at several points adjacent the struts 5 as is indicated at 6.

In Figure 2 the warp and weft of the fabric are indicated by reference numeral 7. When the fireproofing solution is used it impregnates the fabric as is indicated in dotted lines throughout the warp and the weft threads. The fireproof glue layers which are next applied are indicated by the reference letters A and B. C indicates the sealing-in film, layer of pyroxylin, or whatever other waterproofing material may be employed. As many layers of A, B and C as desired may be used as has been described.

The uppermost layer D in Figure 2 indicates the final coating of varnish. Either one or both sides of the fabric may be thus treated.

The same methods of treatment may be usefully applied for the production of other materials intended to resist water or weather and flame, as for instance underwriters' cloth, tents, balloons, etc.

In producing the compound fabric for aeroplane wings it is of course not necessary to seal in the base of the assemblage since the two layers of protected cloth at the top and bottom of the wing protect each other. Where a cloth is to be waterproofed and flame-proofed on both sides it is merely necessary to duplicate the treatment above described with regard to one side. In many articles however, as an underwriters' cloth, it is not desired to waterproof the under side and such materials may be made exactly as above described for an aeroplane wing. Of course thread or yarn may be treated in the manner above described and then formed into a fabric. In this case every thread of the fabric will contain fireproofing salts,

carry a layer of glue or the like and be sealed in by a tenuous layer of waterproofing material. But it is ordinarily easier to treat the fabric itself.

In lieu of the glue more specifically mentioned ante, any other colloid material capable of giving moist strong films may be used in lieu thereof, such as algin, Irish moss, Iceland moss, concentrated waste sulfite liquid, viscose, etc. A good starch size, such as 75 apparatin, is applicable. Such a mixture as is produced by dissolving borax in starch paste is applicable. A mixture of borax, sulfate of alumina and starch gives a good, strong coating material. In using glue or 80 gelatin, I may employ the dry commercial articles; or I may use the liquid materials which are variously known as "size," "glue size," etc. Low grade glues such as those made from stick may be used. As the waterproofing and film forming layer I regard pyroxylin in the form of celluloid or colloidion cotton as best adapted, but a wide variety of other materials may be used, such as cellulose acetate, "bakelite" (a phenol for maldehyde condensation product) etc. Ordinary varnishes are not well adapted since they require too thick a layer to produce impermeability. When pyroxylin is used it may be softened or made flexible by camphor or castor oil in the usual manner; but it should not be loaded with hygroscopic salts as is sometimes done for producing a fireproofing salt.

In making aeroplane wings under the present invention it is highly advantageous to protect the wood itself in the manner hereinbefore stated; that is to impregnate the wood of the framework with fireproofing salts, dry somewhat, coat with a hygroscopic solution, sharply dry and finally waterproof with a pyroxylin film.

In fireproofing aeroplane wings under the present invention, the essential idea is incorporating permanently moist material (with or without ammonia yielding materials, but usually with) in the fabric, part of the water being present as moisture and part as what may be called latent moisture, that is, water of crystallization or constitution, and then sealing in the water and the ammonia with the aid of thin films of something that is not dissolved or be affected by water and is impervious enough to insulate the fireproofing materials against access of air.

In lieu of using glycerin as the hygroscopic agent in the glue etc. layer I may of course use any other hygroscopic agent, as for instance, sugar, molasses, glucose, confectioners' glucose, honey, glycol, etc.

What I claim is:—

1. The process of treating textile materials which comprises impregnating such material with a fireproofing chemical and applying a glue solution containing hygro-

scopic materials, sealing in the treating materials so employed with a thin film of pyroxylin, applying a film of a glue solution, drying and again applying a film of water-  
5 proofing material.

2. The process of treating textile ma-  
terials which comprises impregnating fabric  
with a solution of a fireproofing salt, drying  
somewhat, coating with a glue solution con-  
-10 taining hygroscopic materials, sharply dry-  
ing, treating with a waterproofing solution  
and once more drying.

3. The process of treating textile ma-  
terials which comprises impregnating fabric  
15 with a solution of a fireproofing salt, drying  
somewhat, impregnating with a glue solu-  
tion containing hygroscopic materials,  
sharply drying, treating with a waterproof-  
ing solution, drying, treating with a glue  
20 solution, once more drying and applying an-  
other waterproofing film.

4. The process of treating textile ma-  
terials which comprises impregnating such  
a material with fireproofing chemicals and  
25 an uninflammable size, sealing the impreg-  
nating materials in position by thin films  
of a waterproofing material and finally coat-  
ing the material with a mechanically resis-  
tant coating.

30 5. In the manufacture of aeroplane wings  
the process which comprises treating the  
frames thereof with a fireproofing material,  
stretching and fastening the fabric covering  
on the frames, treating the fabric with a

moist fireproofing material while on the 35  
frames and sealing the same in place by a  
film of waterproofing material.

6. Fabric for aeroplanes and the like im-  
pregnated with a strengthening and water-  
proofing material and carrying a layer of 40  
moist fireproofing material and a water-  
proofing layer sealing it in place.

7. As a new article of manufacture, a tex-  
tile fabric having the threads or fibers im-  
pregnated with fireproofing chemicals and 45  
coated with moist uninflammable water-  
proofing material, and thin films of other  
waterproofing material sealing such chemi-  
cals and first mentioned waterproofing ma-  
terial in place. 50

8. As a new article of manufacture, a tex-  
tile fabric having the threads or fibers im-  
pregnated with fireproofing chemicals and  
coated with a composition containing hy-  
groscopic materials, and a film of water- 55  
proofing material sealing such chemicals and  
such compositions in place.

9. As a new article of manufacture, a tex-  
tile fabric having the threads or fibers im-  
pregnated with fireproofing chemicals and 60  
coated with a composition containing hy-  
groscopic materials, and a plurality of wa-  
terproof films spaced and united by inter-  
vening films of a dried colloid composition  
sealing such chemicals and such hygroscopic 65  
materials in place.

In testimony whereof, I affix my signature.  
GUIDO BLENIO.